

# UNITED STATES PATENT OFFICE.

EDWIN E. GLASKIN, OF LOWER CAPE, NEW BRUNSWICK, CANADA.

## FIRE-KINDLER.

SPECIFICATION forming part of Letters Patent No. 252,757, dated January 24, 1882.

Application filed June 10, 1881. (No specimens.)

*To all whom it may concern:*

Be it known that I, EDWIN EAGLING GLASKIN, of Lower Cape, county of Albert, Province of New Brunswick, Canada, have invented a new and Improved Fire-Kindler; and I do hereby declare that the following is a full and exact description thereof.

My invention is an improvement in the class of fire-kindling blocks containing sawdust, resin, and tallow, or some other oleaginous substance. Such blocks have had two prominent defects, which have greatly impaired their utility—that is to say, they have been either too soft, so as to soon lose their form and adhere together, or too brittle and friable, so that they would not retain their shape, but crumble into fragments. These results are due to lack of due proportion of the ingredients and of sufficient pressure when the blocks are being molded.

My invention remedies said defects and enables me to produce a greatly superior article, it being more firm and dense or compact, less sticky, and yet less friable; also, better adapted for handling and transportation, as well as cheaper and capable of maintaining a flame for a longer time.

To enable others skilled in the art to make and use my invention, I will proceed to describe its construction and operation.

All moisture is first driven out of the sawdust by heat, and after this has been effected I mix therewith powdered resin, continuing to heat and stir until they are thoroughly incorporated. A small quantity of pitch or other coloring matter, if desired, is then added and stirred until incorporation is complete. Finally some tallow, petroleum, still-bottoms, or other oleaginous substance is then added, the heating and stirring being continued uninterrupted

in the meantime and thereafter until all the substances are interspersed among each other. I then form the compound, which is still in a granular condition, while hot, in molds, and

subject it therein to a pressure of about one thousand pounds per square inch.

By my invention I am enabled to produce a tough, solid, homogeneous mass by the admixture of five parts sawdust, one resin, and one-sixteenth of one of tallow or oleaginous substance, and a cake or mold measuring two inches by three inches by one-half inch will keep ablaze from fifteen to twenty minutes, and will kindle a green coal fire without the assistance of wood. Such results have never before been attained, so far as I am aware.

By the means which I employ and above referred to I also make torches and other articles which will support a hot or bright flame for a prolonged period.

I sometimes insert a small block of wood or other combustible substance in the center of each mold or cake for the purpose of spending the other substances.

What I claim as my invention, and desire to secure by Letters Patent, is—

1. The process of producing fire-kindling blocks, which consists in mixing dry sawdust with resin and oil, in the proportions, respectively, of five parts, one part, and one-sixteenth of one part, and then placing the mass in suitable molds and compressing it to the degree of one thousand pounds, or thereabout, to the square inch for the purpose of compacting it into hard non-friable blocks, as set forth.

2. As an improved article of manufacture, a fire-kindling block composed of five parts sawdust, one part resin, and one-sixteenth part oil mixed together and densely compacted, so that the block is hard and non-friable, as specified.

Lower Cape, Hopewell, Albert county, New Brunswick, Canada.

EDWIN EAGLING GLASKIN.

In presence of—

S. G. MORSE,  
REB. C. PECK.